

## UNITED STATES PATENT OFFICE

2,026,531

## PROPELLENT POWDER

George C. Hale and Donald R. Cameron,  
Dover, N. J.No Drawing. Application March 20, 1934,  
Serial No. 716,512

2 Claims. (Cl. 52—13)

(Granted under the act of March 3, 1883, as  
amended April 30, 1928; 370 O. G. 757)

The invention described herein may be manufactured and used by or for the Government for governmental purposes, without the payment to us of any royalty thereon.

5 This invention relates to a propellant powder.

The requirements of a propellant powder for military weapons are low volatility, resistance to moisture absorption and chemical decomposition, smokelessness, and flashlessness.

10 It is recognized by those experienced in the preparation of propellant powders that no powder has been produced to date which fulfills all the requirements above cited to the desired degree under all circumstances. Thus a particu-

15 lar powder may be acceptable for use because it offers advantages in fulfilling one or more of the requirements above mentioned even though it does not offer any particular advantage with respect to other of the requirements, but al-  
though acceptable, such a powder is obviously  
20 not all that is to be desired.

One of the principal difficulties in preparing powders which yield no flash at the muzzle of guns resides in the fact that the common methods of eliminating flash involve the addition to the powder composition of ingredients which have the objectionable tendency of producing smoke when the powder is fired. The user is, therefore, confronted with the problem of choosing between a powder which flashes but produces a minimum of smoke and a powder which is flashless but produces more smoke than is really desired.

25 The purpose of this invention is to provide a non-hygroscopic, non-volatile and stable nitrocellulose propellant powder which is absolutely flashless and produces less smoke than powders heretofore in use. This purpose is accomplished by incorporating in the powder composition a relatively small amount of triacetin. The triacetin is the pure product or mixtures of it with small amounts of diacetin and monoacetin such as are obtainable commercially under the name triacetin.

30 It has been found by firing powders made from compositions containing nitrocellulose and triacetin that the triacetin is very efficient in reducing the flash from the nitrocellulose powders and at the same time yields only a thin, fugitive smoke which is decidedly less visible than that produced by any other flashless powders.

35 While satisfactory powders for some uses can be produced from compositions containing only nitrocellulose, triacetin and the commonly used stabilizer diphenylamine, it has been found that

powders that are more widely adaptable can be obtained by the addition of trinitrotoluene to the composition. Examples of compositions are given which have been thoroughly tested in 37m/m and 75m/m military weapons and found to be not merely satisfactory but distinctly su-  
perior to other flashless powders from the stand-  
point of the amount of smoke produced when flashlessness is consistently obtained:

|                 | Per cent |
|-----------------|----------|
| Nitrocellulose  | 80       |
| Trinitrotoluene | 15       |
| Triacetin       | 5        |
| Nitrocellulose  | 80       |
| Trinitrotoluene | 10 15    |
| Triacetin       | 10       |

These compositions are cited as representative but not limiting since various proportions of the three constituents have been employed in pow-  
ders and their relative behavior established. It  
is to be understood that variations in the pro-  
portion of the constituents are necessary when  
adapting the powders to specific weapons since  
the optimum proportion for one weapon may  
not be the optimum for another weapon. It is  
clearly recognized by those experienced in the  
preparation of propellant powders that the prob-  
lem of eliminating flash is much greater with  
some weapons than others. The length of the  
tube or barrel of the gun is one factor since a  
long tube permits greater radiation of heat from  
the gases before they issue from the muzzle and  
it is therefore easier to reduce the temperature  
of the gases below their inflammation tempera-  
ture by the flash reducing agent employed in the  
powder. Thus with some weapons which have  
a long tube and require a relatively small amount  
of propellant powder to meet ballistic require-  
ments, the addition of 2% triacetin may be suf-  
ficient to eliminate flash while with a gun or  
howitzer which has a short tube and requires a  
much larger amount of propellant charge, 5%  
or even 10% of the triacetin may be needed. If  
the percent of this constituent is varied the per-  
centage of the nitrocellulose or trinitrotoluene  
must of course be changed accordingly.

We claim:

1. A propellant powder consisting of nitrocel-  
lulose, trinitrotoluene and triacetin two to ten  
per cent.
2. A propellant powder consisting of nitrocel-  
lulose, trinitrotoluene and triacetin.

GEORGE C. HALE.

DONALD R. CAMERON. 55